

# United States Patent [19]

Schumacher et al.

[11] 4,099,967  
[45] Jul. 11, 1978

[54] **GALLING RESISTANT AUSTENITIC STAINLESS STEEL**

[75] Inventors: **William J. Schumacher; Harry Tanczyn**, both of Baltimore, Md.

[73] Assignee: **Armco Steel Corporation**, Middletown, Ohio

[21] Appl. No.: **751,022**

[22] Filed: **Dec. 14, 1976**

[51] Int. Cl.<sup>2</sup> ..... C22C 38/02; C22C 38/58

[52] U.S. Cl. ..... 75/128 A; 75/128 C

[58] Field of Search ..... 75/128 A, 128 C; 148/38

[56] **References Cited**

**U.S. PATENT DOCUMENTS**

|           |         |                   |       |          |
|-----------|---------|-------------------|-------|----------|
| 2,984,563 | 5/1961  | Tanczyn           | ..... | 75/128 C |
| 3,615,368 | 10/1971 | Baumel            | ..... | 75/128 C |
| 3,663,215 | 5/1972  | Tanczyn           | ..... | 75/128 C |
| 3,785,787 | 1/1974  | Yokota et al.     | ..... | 75/128 C |
| 3,806,337 | 4/1974  | Jones             | ..... | 75/128 C |
| 3,900,316 | 8/1975  | Jones             | ..... | 75/128 C |
| 3,912,503 | 10/1975 | Schumacher et al. | ..... | 75/128 A |
| 4,002,510 | 1/1977  | Wilde             | ..... | 75/128 G |

**FOREIGN PATENT DOCUMENTS**

1,275,007 5/1972 United Kingdom ..... 75/128 C

**OTHER PUBLICATIONS**

Steel Products Manual, 12/1974, pp. 21-22.

*Primary Examiner*—Arthur J. Steiner  
*Attorney, Agent, or Firm*—Melville, Strasser, Foster & Hoffman

[57] **ABSTRACT**

An austenitic stainless steel which in wrought or cast, and annealed, condition exhibits excellent galling resistance, excellent stress corrosion resistance in chloride-containing environments, good resistance against inter-granular corrosion, good high temperature oxidation resistance, and a high work hardening rate. The broad composition range is, in weight percent, about 13 to about 19% chromium, about 13 to about 19% nickel, 0.5 to about 4% manganese, 3.5 to about 7% silicon, up to about 0.15% carbon, less than 0.04% nitrogen, about 0.05% maximum phosphorus, about 0.05% maximum sulfur, and balance essentially iron except for incidental impurities. The steel can be readily worked with conventional equipment and has particular utility for applications in which moving metal-to-metal contact, corrosive attack and/or elevated temperature are encountered in combination. The steel can also be cast into articles of ultimate use, or utilized in powder metallurgy techniques.

**2 Claims, No Drawings**

## GALLING RESISTANT AUSTENITIC STAINLESS STEEL

### BACKGROUND OF THE INVENTION

#### (1) Field of the Invention

This invention relates to an austenitic stainless steel exhibiting the combination of excellent galling resistance in conventional wrought and annealed form, excellent stress corrosion resistance in chloride-containing environments, good resistance against intergranular corrosion, good high temperature oxidation resistance, good wear resistance, and a high work hardening rate. The alloy of this invention can be readily worked with conventional equipment into plate, sheet, strip, bar, rod and the like, and retains a substantially austenitic structure throughout a wide temperature range.

The steel of the invention is adapted to applications in which moving metal-to-metal contact, corrosive attack and/or high temperatures are encountered in combination. Although not so limited, the steel has particular utility for fabrication into roller chains, link belts on conveyors, valves subjected to elevated temperature, woven metal belts for continuous heat treating furnaces, fasteners, pins and bushings.

#### (2) Description of the Prior Art

Although galling and wear may occur under similar conditions, the types of deterioration involved are not similar. Galling may be defined as the development of a condition on a rubbing surface of one or both contacting metal parts wherein excessive friction between minute high spots on the surfaces results in localized welding of the metals at these spots. With continued surface movement this results in the formation of even more weld junctions which eventually sever in one of the base metal surfaces. The result is a build-up of metal on one surface, usually at the end of a deep surface groove. Galling is thus associated primarily with moving metal-to-metal contact and results in sudden catastrophic failure by seizure of the metal parts.

On the other hand, wear is synonymous with abrasion and can result from metal-to-metal contact, or metal-to-non-metal contact, e.g. the abrasion of steel mining equipment by rocks and similar mineral deposits. Such wear is characterized by relatively uniform loss of metal from the surface, as contrasted to localized grooving with consequent metal build-up, as a result of rubbing a much harder metallic surface against a softer metallic surface. The distinction between galling and wear can perhaps best be illustrated by the fact that galling can be eliminated by mating or coupling a very hard metallic surface with a much softer metallic surface, whereas wear or abrasion in metal-to-metal contact would be increased by mating a very hard surface with a much softer one.

An article by Harry Tanczyn entitled "Stainless Steel Galling Characteristics Checked" in *STEEL*, Apr. 20, 1954 points out that stainless steel sections at a relatively high hardness level, or with a substantial difference in hardness, exhibit better resistance to galling than the combination of two soft members. This may be explained by the theory that the hardened sections deform elastically near the contact points under loading, while the softer pieces yield plastically for a significant distance beneath the contact points. During movement, the hardened surfaces apparently recover elastically with decrease in pressure, and this motion tends to sever any metallic welding. This article also indicates that

good resistance to galling may be traceable to the combination of a suitable oxide surface film and a hard backing. Oxide films were found to influence the galling characteristics of metals, e.g. a film of  $Fe_3O_4$  increased the resistance of mild steel to galling, while a film of  $Fe_2O_3$  did not benefit resistance to galling.

Among the numerous prior art steels currently available, the austenitic AISI Type 304 is suited to a variety of uses involving welding and fabrication, but the galling and wear resistance of this steel are poor, and the metal is likely to fail when subjected to such conditions.

A precipitation-hardening stainless steel, sold under the registered trademark ARMCO 17-4 PH (about 15.4% chromium, about 4.0% nickel, about 4.0% copper, about 1.0% manganese, about 1.0% silicon, up to 0.07% carbon, 0.35% columbium, and remainder iron), while possessing high strength and hardness in the hardened condition, exhibits only fair galling and wear resistance.

U.S. Pat. No. 3,663,215, issued May 16, 1972 to H. Tanczyn, discloses a steel having improved wear resistance, which at the same time is weldable, workable, and/or machinable, and precipitation hardenable by heat treatment to great hardness. It has been found that this steel has good galling resistance. However, it contains large amounts of expensive alloying elements, and it is difficult to process with standard steel mill equipment. The broad composition ranges are about 10 to about 22% chromium, about 14 to about 25% nickel, about 5 to about 12% silicon, one or more of the elements molybdenum up to about 10%, tungsten up to about 8%, vanadium up to about 5%, columbium up to about 5% and titanium up to about 5%, these additional elements being in sum total of about 3 to about 12%. Carbon is present up to about 0.15% and nitrogen up to about 0.05%. In this alloy silicon is stated to form silicides of molybdenum, tungsten and the like, in finely dispersed form in the matrix of the precipitation-hardened steel. These silicides are of extreme hardness, thereby providing good wear resistance.

A prior art steel presently considered to have the best resistance to wear and galling is the straight chromium AISI Type 440C, containing about 16 to 18% chromium, about 1% maximum manganese, about 1% maximum silicon, about 0.75% maximum molybdenum, about 0.95 to 1.20% carbon, and remainder iron. This steel is hardenable by heat treatment but has poor corrosion resistance and poor formability. It is difficult to roll into plate, strip, sheet, bar or rod, and articles of ultimate use cannot be readily fabricated from plate, sheet, strip, bar or rod form.

U.S. Pat. No. 2,177,454, issued Oct. 24, 1939 to H. L. Frevert et al, discloses a valve steel for use in internal combustion engines, preferably containing from 0.10 to 1.0% carbon, over 10% and less than 20% chromium, 5 to 13% manganese plus nickel, the manganese being over 3% and less than 10.25% and nickel being over 1.75% and not over 3.5%, with the manganese content substantially exceeding the nickel content, 2.5 to 4.5% silicon or aluminum, the silicon being over 1.25%, and balance substantially iron.

U.S. Pat. No. 3,615,368, issued Oct. 26, 1971 to A. Baumel, discloses an austenitic steel alleged to have high resistance to stress crack corrosion and to solutions of nitric acid, containing up to 0.25% carbon, 1.5 to 10% silicon, up to 10% manganese, 13 to 30% chromium, 4 to 30% nickel, up to 10% molybdenum, 0.04 to 0.3% nitrogen, and balance iron and unavoidable impu-

rities. The addition of nitrogen in an amount of 0.04 to 0.3%, and preferably from 0.08 to 0.2%, is stated to minimize formation of intermetallic deposits at the grain boundaries of the heat affected zone of a weld.

Reference is further made to U.S. Pat. No. 3,912,503 issued Oct. 14, 1975 to the present applicants and assigned to the assignee of the present application. The patent discloses an austenitic stainless steel having excellent galling resistance in conventional wrought form, good wear resistance, good corrosion resistance in chloride-containing environments, and a high work hardening rate. The steel of this U.S. patent consists essentially of from about 10 to about 25% (preferably about 12 to about 19%) chromium, about 3% to about 15% (preferably about 4 to about 12%) nickel, about 6 to about 16% (preferably about 7 to about 13%) manganese, about 2 to about 7% (preferably 3 to 5%) silicon, about 0.001 to about 0.25% (preferably about 0.01 to about 0.12%) carbon, about 0.001 to about 0.4% (preferably about 0.03 to about 0.3%) nitrogen, up to about 4% (preferably about 0.75% maximum) molybdenum, up to about 4% (preferably about 0.75% maximum) copper, a maximum of about 0.09% phosphorus, a maximum of 0.25% sulfur, a maximum of 0.50% selenium, and remainder essentially iron except for incidental impurities.

In our above-mentioned U.S. Pat. No. 3,912,503 the silicon addition is believed to modify the composition of the surface oxide film of the steel, making it more stable and adherent. Silicon is dissolved in an austenitic matrix. Moreover, the silicon addition exerts a substantial increase in the work hardening rate of the steel. Unlike the steel of the above mentioned U.S. Pat. No. 3,663,215, silicon does not form a silicide of molybdenum, tungsten, vanadium, columbium and/or titanium.

### SUMMARY

It is the object of the present invention to provide an austenitic stainless steel having, in combination, excellent galling resistance in wrought or cast form, excellent stress corrosion resistance in chloride-containing environments, excellent resistance against intergranular corrosion, good high temperature oxidation resistance, good wear resistance and a high work hardening rate, which is at the same time readily workable into plate, sheet, strip bar, rod, tube, pipe, and like wrought products. The steel is also adapted to powder metallurgy applications, and surface coatings including those made by powder-filled tube forms and the plasma arc process.

In its broad ranges the steel of the present invention consists essentially of, in weight percent, about 13 to about 19% chromium, about 13 to about 19% nickel, 0.5 to about 4% manganese, 3.5 to about 7% silicon, up to about 0.15% carbon, less than 0.04% nitrogen, about 0.05% maximum phosphorus, about 0.05% maximum sulfur, and balance iron except for incidental impurities. More specifically, impurities such as molybdenum, copper, tungsten, columbium, vanadium and titanium are restricted to residual amounts.

The elements silicon, chromium, nickel, manganese and nitrogen, and the balance therebetween are critical in every sense. Omission of one of the essential elements, or departure from the ranges set forth above, results in loss of one or more of the desired properties.

The silicon content of the steel of the present invention is of particular criticality. Although not bound by theory, it is believed that silicon (within the range of 3.5 to 7%, and preferably from 4 to 5.5%), performs the same dual function in the present steel as explained

above with respect to the steel of our U.S. Pat. No. 3,912,503. More specifically, the effect of silicon in conferring galling resistance and internal strain-or work-hardening is dependent on the silicon being dissolved in an austenitic matrix. This effect is not obtained in a ferritic phase.

A minimum of 3.5% and preferably about 4.0% silicon is needed for this effect. A maximum of 7% silicon and preferably a maximum of about 5.5%, must be observed for good workability and formability, and also to assure an austenitic structure.

At least 13% chromium is required for corrosion resistance and high temperature oxidation resistance. However, a maximum of 19% chromium must be observed in order to insure an austenitic structure at minimum nickel levels. Chromium has little influence on the strain hardening rate.

Nickel is necessary in the amount of at least 13% in order to obtain an austenitic structure. Since silicon is a potent ferrite former, at least about 13% nickel is needed to offset this effect. However, a maximum of about 19% nickel must be observed since greater amounts adversely affect galling resistance and decrease the strain or work hardening rate.

A minimum of 0.5% manganese is needed to stabilize the austenitic structure and to provide a high strain hardening rate. More than 4% manganese provides no additional benefit in achieving these functions.

Nitrogen must be restricted to less than 0.04% by weight for best galling resistance and resistance against intergranular corrosion (i.e. low Huey rate) in the reheated condition, as will be shown hereinafter. The relatively high silicon range of the steel of the present invention greatly restricts nitrogen solubility. A purposeful addition of nitrogen thus would result in the danger of porosity, i.e. gassy heats, in the as-cast steel.

Contrary to the steel of the above mentioned U.S. Pat. No. 3,663,215, silicides of molybdenum, tungsten, vanadium, columbium and/or titanium are not relied upon to impart wear resistance. Surprisingly, elimination of these elements from the steel of the present invention (i.e. restriction to residual amounts) results in a marked improvement in galling resistance, the theoretical basis for which has been explained hereinabove. Moreover, omission of molybdenum, tungsten, vanadium and the like results in an improvement in the hot and cold workability of the steel of this invention on conventional mill equipment. Since these elements are ferrite formers, introduction thereof would require additional nickel with consequent higher cost.

### DESCRIPTION OF THE PREFERRED EMBODIMENTS

While the broad composition set forth above exhibits the novel combination of properties which is the primary object of the invention, optimum stress corrosion resistance in chloride-containing environments is achieved by observance of the following preferred ranges, all percentages being by weight:

|            |                                |
|------------|--------------------------------|
| Chromium   | about 14% to about 16%         |
| Nickel     | about 14% to about 17%         |
| Manganese  | about 0.5% to about 3.0%       |
| Silicon    | about 4.0% to about 5.5%       |
| Carbon     | about 0.03% to about 0.10%     |
| Nitrogen   | about 0.03% maximum            |
| Phosphorus | about 0.05% maximum            |
| Sulfur     | about 0.05% maximum            |
| Iron       | balance, except for incidental |

## -continued

impurities.

As in the broad composition, the preferred composition also restricts the elements molybdenum, copper, tungsten, columbium, vanadium and titanium to residual amounts.

The elements silicon and manganese act to lower the stacking fault energy at the planes of atom disarray within the annealed austenitic matrix of the steel of the invention. Under mechanical loading, the lowered stacking fault energy promotes the development of numerous stacking faults in the face-centered cubic annealed austenitic microstructure. When a stacking fault forms, it is equivalent to producing locally several layers of a hexagonal close-packed structure. The strain-hardening rates of faulted structures are much greater than those of unfaulted structures, i.e., a multiplication factor is introduced. In addition, the frictional forces at surface contact points for hexagonal close-packed structures are markedly lower than those for face-centered cubic structures. Moreover, in the present steel silicon atoms diffuse rapidly to points or planes of stress (viz., contact surfaces), thereby achieving excellent galling resistance.

The function of silicon in increasing the work hardening or strain-aging rate of the steel of the invention is somewhat offset by the nickel addition, since an increase in the nickel content tends to lower slightly the work hardening rate of the steel by increasing the stacking fault energy. However, an increase in the silicon content within the range set forth above results in a net increase in the work hardening rate. Preferably nickel is varied directly in proportion to the silicon content in order to offset the ferrite forming tendencies of silicon, without unduly lowering the work hardening rate of the steel.

Carbon is of course present and a maximum of 0.15% should be observed since silicon directly limits carbon solubility in ferrous-base alloys. Precipitation of carbon as carbides tends to produce a ferro-magnetic condition, which should be avoided in the steel of the invention. Preferably, a minimum of about 0.03% carbon is present for its function in strengthening the steel and in contributing to an austenitic structure. For best stress corrosion resistance the carbon preferably is restricted to a maximum of about 0.10%.

## EXAMPLE 1

An experimental heat has been prepared falling within the above preferred composition ranges and subjected to stress corrosion resistance, high temperature oxidation resistance and galling resistance tests. The heat was melted, cast in conventional manner, hot forged to  $\frac{1}{2}$  inch round corner squares, annealed at 1093° C for  $\frac{1}{2}$  hour and water quenched. This heat (hereinafter designated as Example 1) had the following composition in weight percent:

|            |                                |
|------------|--------------------------------|
| Chromium   | 15.27%                         |
| Nickel     | 15.69%                         |
| Manganese  | 0.80%                          |
| Silicon    | 4.76%                          |
| Carbon     | 0.063%                         |
| Nitrogen   | 0.03%                          |
| Phosphorus | residual                       |
| Sulfur     | residual                       |
| Iron       | balance, except for incidental |

## -continued

impurities.

5 Stress corrosion tests on specimens of the above heat and comparative tests on a specimen of AISI Type 304 (0.08% max. carbon, 2.00% max. manganese, 18.00 – 20.00% chromium, 8.00 – 12.00% nickel) were conducted in boiling magnesium chloride solution of 42% concentration at varying tensile stresses and are set forth in Table I. It is apparent that the steel of the present invention is far superior in stress corrosion resistance in chloride-containing environments to Type 304, despite the unexplained premature failure of the specimen of Example 1 at 45 ksi. The results at stresses of 50 and 60 ksi indicate that the test at 45 ksi should not be considered typical.

TABLE I

| Stress (ksi) | Stress Corrosion Resistance<br>Boiling MgCl <sub>2</sub> (42%) |                             |
|--------------|----------------------------------------------------------------|-----------------------------|
|              | Example 1<br>(Steel of Invention)                              | Type 304                    |
| 40           | 285.6                                                          | 0.9                         |
| 45           | 40.7                                                           | 0.8                         |
| 50           | 99.2                                                           | (average of<br>2 tests) 0.6 |
| 60           | 110.1                                                          | 0.4                         |

30 Static and cyclic high temperature oxidation tests were conducted on the steel of Example 1 in comparison with specimens of AISI Type 304 and AISI Type 310. These tests are reported in Table II. The cyclic test results are considered more significant than the static test results, and it is evident that the steel of the invention exhibits far greater oxidation resistance than Type 304 and is comparable in oxidation resistance to the highly alloyed Type 310 (0.25% max. carbon, 2.00% max. manganese, 24.00 – 26.00% chromium, 19.00 – 22.00% nickel). In this connection, it should be noted that Type 310 is generally recommended for applications requiring good high temperature strength and oxidation resistance.

TABLE II

|                                  | Oxidation Resistance              |             |             |
|----------------------------------|-----------------------------------|-------------|-------------|
|                                  | Weight loss (mg/cm <sup>2</sup> ) |             |             |
|                                  | Example 1<br>(Steel of Invention) | Type<br>304 | Type<br>310 |
| Static                           |                                   |             |             |
| 240 hrs. at 1093° C              | 158                               | 2265        | 21          |
| Cyclic                           |                                   |             |             |
| 1288°-871° C/R.m.T.<br>27 cycles | 10                                | 1064        | 21          |
| 1065°-830° C/R.m.T.<br>55 cycles | 14                                | 361         | 10          |

55 The annealed bar stock of Example 1 was subjected to galling resistance tests against itself and against a number of prior art alloys. For purposes of comparison each of four of the prior art alloys was tested against itself, and AISI Type 304 was tested against the same 60 prior art alloys as Example 1. Test results are set forth in Table III.

The test method utilized in obtaining the data of Table III comprised rotation of a polished cylindrical section or button for one revolution under pressure against a polished block surface in a standard Brinell hardness machine. A button specimen was prepared by drilling a countersunk hole to accommodate most of the exposed Brinell hardness ball, the specimen then being

mounted in Bakelite and polished to a 600 grit finish in a Buehler Automet Unit to obtain a relatively flat test surface, with the edges slightly rounded. The button was then broken out of the Bakelite, and the edges were hand deburred. A block specimen was ground parallel on two sides and hand-polished to a 3/0 emery grit finish, equivalent to a 600 grit finish. Both the button and block specimens were degreased by wetting with acetone, and the hardness ball was lubricated just prior to testing. The button was hand-rotated slowly at a predetermined load for one revolution and examined for galling at 10 $\times$  magnification. If galling was not observed (i.e. absence of metal build-up, usually at the end of a groove), a new button and block area couple was tested at successively higher loads until galling was first observed. Confirmation was obtained by testing one more coupling or combination at a higher load. Since light loads did not cause full area contact due to the rounded button edges, the actual contact area was measured at 10 $\times$  to convert to galling stress.

In Table III the button specimen is the first alloy mentioned in each couple, and the second alloy is the block specimen. It will be noted that several couples of Example 1 with prior art alloys reached the limits of the test equipment without exhibiting galling so that the true galling stress of these samples was not actually determined.

It is apparent from the data of Table III that the steel of the present invention exhibits excellent galling resistance when rotated against itself, and without exception exhibits substantially higher galling resistance than AISI Type 304 when rotated against the same prior art alloy. It is significant to note that AISI Type 440C, presently considered to have the best resistance to galling and wear, exhibited a galling stress of 11 ksi when rotated against itself, and hence is substantially inferior in galling resistance to the steel of the present invention when rotated against itself.

Hardness values for the various alloys subjected to galling resistance tests were not determined, but it was observed empirically that the initially hardness of the

TABLE III-continued

| Couple                 | Galling Resistance<br>Unlubricated Tests |                      | Galling Stress (ksi) |
|------------------------|------------------------------------------|----------------------|----------------------|
|                        | Example 1 v. AISI 410                    | AISI 304 v. AISI 410 |                      |
| Example 1 v. AISI 303  | 18                                       | 2                    |                      |
| AISI 304 v. AISI 303   | 2                                        | 2                    |                      |
| Example 1 v. AISI 304N | 37.7+                                    | 2                    |                      |
| AISI 304 v. AISI 304N  | 39.2+                                    | 2                    |                      |
| Example 1 v. AISI 201  | 55.6+                                    | 3                    |                      |
| AISI 304 v. AISI 201   | 55.6+                                    | 3                    |                      |
| Example 1 v. AISI 440C |                                          |                      |                      |
| AISI 304 v. AISI 440C  |                                          |                      |                      |

+ = Reached practicable load limit of test machine without galling

Further galling resistance tests were conducted on several experimental alloys somewhat similar in composition to the steel of the invention but departing therefrom in one or more of the essential elements. The compositions of these alloys, and galling resistance of each rotated against itself by the above described test method are set forth in Table IV.

A comparison of Sample 2 with Sample 3 (3.3% and 4.2% silicon, respectively) indicates that a minimum of about 3.5% silicon is necessary for excellent galling resistance.

A comparison of Samples 4 and 5 with Sample 3 indicates that when chromium and nickel each exceed 19%, galling resistance is drastically decreased, regardless of silicon contents.

Sample 6 is within the broad ranges of the steel of the invention except for the nitrogen content. It is apparent that the nitrogen level of 0.05% adversely affected the galling resistance.

Accordingly, the silicon, chromium, nickel and nitrogen ranges of the steel of the present invention must be considered critical from the standpoint of galling resistance. The presence of tungsten in Samples 4 and 5 apparently also contributed to the poor galling resistance, although tungsten is substantially neutral with respect to austenite stability when the alloy undergoes work-hardening.

TABLE IV

| Sample | COMPOSITIONS-WEIGHT PERCENT |      |      |       |       |     |     | Galling<br>Stress (ksi)<br>v. itself |
|--------|-----------------------------|------|------|-------|-------|-----|-----|--------------------------------------|
|        | C                           | Mn   | Si   | Cr    | Ni    | N   | W   |                                      |
| 2      | .078                        | 8.0  | 3.3  | 16.2  | 5.0   | .03 | nil | 27                                   |
| 3*     | .070                        | 7.8  | 4.2  | 16.0  | 6.0   | .04 | nil | 42+                                  |
| 4      | .04                         | 0.5  | 3.37 | 20.0  | 20.0  | .04 | 3.5 | 3                                    |
| 5      | .04                         | 0.5  | 4.2  | 20.0  | 20.0  | .04 | 3.5 | 3                                    |
| 6      | .031                        | 0.73 | 5.54 | 15.11 | 15.46 | .05 | nil | 25                                   |

+ = Reached limit of test machine without galling

\* = Steel of preferred composition of applicant' Pat. No. 3,912,503

In the above Samples 2-6, the balance was iron and incidental impurities.

steel of Example 1 was substantially less than that of Type 440C. Despite the high hardness of Type 440C, its galling resistance against itself and against AISI Type 304 was substantially lower than that of the steel of the invention.

TABLE III

| Couple                 | Galling Resistance<br>Unlubricated Tests |                      | Galling Stress (ksi) |
|------------------------|------------------------------------------|----------------------|----------------------|
|                        | Example 1 v. Example 1                   | AISI 304 v. AISI 304 |                      |
| AISI 316 v. AISI 316   | 4                                        | 3                    |                      |
| AISI 410 v. AISI 410   | 11                                       | 12                   |                      |
| AISI 440C v. AISI 440C | 2                                        |                      |                      |
| Example 1 v. AISI 316  |                                          |                      |                      |
| AISI 304 v. AISI 316   |                                          |                      |                      |

It is therefore evident from the above data that this invention provides an austenitic stainless steel having excellent galling resistance, excellent stress corrosion resistance in chloride-containing environments and good high temperature oxidation resistance.

With respect to intergranular corrosion resistance, particularly at elevated temperature, it has been found that restriction of the nitrogen content to less than 0.04% is critical. Although the previously mentioned Baumel U.S. Pat. No. 3,615,368 alleges that a purposeful nitrogen addition within the range of 0.04 to 0.3% and preferably from 0.08 to 0.2%, retards "the formation of intermetallic deposits at the grain boundaries in steels of this type at temperatures of about 850° C," and reduces or avoids "increased corrosion adjacent to the seam

weld", applicants have conducted tests which prove that in fact the nitrogen addition which is the novel feature of the Baumel patent actually increases the extent of intergranular precipitates even with as little as a 5-minute reheating period at about 850° C. These increased grain boundary precipitates result in low ductil-

5 that Sample 7 exhibited thin, discontinuous intergranular precipitates while Sample 8 exhibited thick, continuous grain boundary precipitates. This accounts for the marked differences in intergranular corrosion resistance, and also indicates that the steel of the invention possesses excellent welding characteristics.

TABLE VI

## INTERGRANULAR CORROSION RESISTANCE

| Heat Treatment                                          | Huey Test<br>ASTM A-262<br>Practice C* | HNO <sub>3</sub> -HF TEST<br>ASTM A-262<br>Practice D**<br>Wt. percent |
|---------------------------------------------------------|----------------------------------------|------------------------------------------------------------------------|
| Sample 7 Annealed 1100° C-1/2hr.-W.Q.                   | .0022                                  | .630                                                                   |
| Sample 7 Annealed and reheated 850° C<br>1 minute-W.Q.  | .0041                                  | .563                                                                   |
| Sample 7 Annealed and reheated 850° C<br>5 minute-W.Q.  | .0040                                  | .372                                                                   |
| Sample 7 Annealed and reheated 850° C<br>30 minute-W.Q. | .0045                                  | .476                                                                   |
| Sample 7 Annealed and reheated 850 20 C<br>2 hour-W.Q.  | .0047                                  | .368                                                                   |
| Sample 7 Annealed and reheated 850° C<br>4 hour-W.Q.    | .0047                                  | .396                                                                   |
| Sample 8 Annealed 1100° C-1/2hr.-W.Q.                   | .0026                                  | .693                                                                   |
| Sample 8 Annealed and reheated 850° C<br>1 minute-W.Q.  | .0130                                  | 4.62                                                                   |
| Sample 8 Annealed and reheated 850° C<br>5 minute-W.Q.  | .0115                                  | 3.89                                                                   |
| Sample 8 Annealed and reheated 850° C<br>30 minute-W.Q. | .0143                                  | 3.08                                                                   |
| Sample 8 Annealed and reheated 850° C<br>2 hour-W.Q.    | .0118                                  | 1.88                                                                   |
| Sample 8 Annealed and reheated 850° C<br>4 hour-W.Q.    | .0148                                  | 2.25                                                                   |

\*Average of two 48-hour periods.

\*\*One 2-Hour period.

ity, lower notch-impact toughness, susceptibility to cracking during welding and during annealing of prior cold worked products, as well as a decrease in galling resistance as shown above in Sample 5 of Table IV. Of still greater significance, the increase in the extent of 35 grain boundary precipitates resulting from a nitrogen addition of 0.04% or more decreases resistance to intergranular corrosion after exposure to elevated temperature (particularly about 850° C.)

Two heats were prepared and subjected to comparative testing. The compositions of these heats are set forth in Table V, and heat treatments and corrosion test results are set forth in Table VI.

TABLE V

| Sample | COMPOSITION-WEIGHT PERCENT |     |     |      |       |      |
|--------|----------------------------|-----|-----|------|-------|------|
|        | C                          | Mn  | Si  | Cr   | Ni    | N    |
| 7      | .032                       | .70 | 3.7 | 18.9 | 15.55 | .033 |
| 8      | .033                       | .78 | 3.9 | 18.5 | 15.29 | .15  |

In Samples 7 and 8, phosphorus was 0.008%, sulfur not greater than 0.025%, and balance iron.

Bar stock from Samples 7 and 8 was annealed by water quenching from 1100° C (after 30 minutes), and individual annealed specimens,  $\frac{1}{8}$  inch round by  $\frac{1}{8}$  inch long, were reheated at 850° C for periods of time set forth in Table VI. These specimens were then subjected to the Huey Test-ASTM A-262 Practice C, and to the Nitric-Hydrofluoric Acids Test-ASTM A-262-68 Practice D. The values of Table VI were averages of duplicate tests. The Huey rates were measured in inches per month, and the HNO<sub>3</sub>-HF rates in percent weight loss.

It is evident that the Huey rates and HNO<sub>3</sub>-HF rates of Sample 7 (0.033% nitrogen), a steel of the present invention, are good even after reheating for 4 hours, whereas those of Sample 8, which differed substantially only in the nitrogen content of 0.15%, were unacceptably high. Metallographic examination of etched heat treated specimens (at 500X magnification) confirmed

45 In the annealed condition, wrought products of the steel of the invention are sufficiently ductile to permit ready fabrication into chains, valves, woven metal belts, fasteners of various types and other articles of ultimate use where metal-to-metal contact under stress would be encountered either at ambient or elevated temperatures. The steel of the invention can readily be welded or brazed and may be cut, drilled, tapped, threaded and machined in other manner in the fabrication of articles of ultimate use.

50 The steel of the invention may be melted in any conventional manner, for example in an induction furnace, and may then be cast into ingots or continuously cast, hot reduced in standard mill equipment to strip, sheet, bar or rod form, annealed, and if desired, cold reduced. Annealing of the hot reduced and/or cold reduced material at about 980° to 1095° C for  $\frac{1}{2}$  hour restores sufficient ductility to permit further fabrication.

55 Alternatively, the molten steel may be cast into articles of ultimate use, the only limitation being that such articles have a size or mass which will permit annealing thereof in conventional equipment.

The steel may also be comminuted into particulate 55 form suitable for powder metallurgy processing into compacted, pressed and/or sintered products, by techniques such as atomizing a melt.

60 Steel having the broad composition of the invention has utility in welding, overlay of metallic surfaces, and like applications. For such uses the steel may be produced in the form of wire or sheet, or in the form of powder-filled tube-like articles. In the case of filled tube articles part of the alloying elements may be contained in the tube-like covering rather than in the powdered metal, and the compositions and proportions will be so selected that upon melting, as in a welding or overlay operation, a composition will be obtained which is within the broad limits of the invention and which,

upon solidification, will be substantially fully austenitic. As a weld filler material the steel may be used to join stainless steels of different or similar compositions.

Plate, sheet, strip, bar, rod, tube, pipe, and like wrought products, metal powder and powder filled tube forms, as well as wrought or cast articles of ultimate use, having the preferred compositions of the present invention, exhibit in the annealed condition a galling resistance of at least 40 ksi stress when rotated against itself in the test method set forth above, a stress corrosion resistance of greater than about 90 hours to failure at 50-60 ksi stress in boiling  $MgCl_2$  (42% concentration) determined by the above test method, and a weight loss not exceeding about 20 mg/cm<sup>2</sup> by the cyclic oxidation resistance test method set forth above. Moreover, steel of the broad and preferred compositions of the invention, in the annealed condition, exhibits a loss of not greater than 0.005 inches per month after reheating at 850° C for periods of time up to 4 hours, by the Huey Test. Regardless of any accepted standards which may exist, no prior art alloy meets all the above test values, to the best of applicants' knowledge.

While certain preferred embodiments of the invention have been specifically disclosed and described, it should be understood that the invention is not so limited, since many variation will be apparent to those skilled in the art, and the invention is to be given its broadest interpretation within the terms of the following claims.

The embodiments of the invention in which an exclusive property or privilege is claimed are defined as follows:

5 1. Austenitic stainless steel having a galling resistance of at least 40 ksi stress when rotated against itself by the test described herein, a stress corrosion resistance of greater than 90 hours to failure at 50-60 ksi stress in boiling magnesium chloride (42% concentration), a Huey rate of not greater than 0.005 inches per month after reheating at 850° C for a time up to four hours, and good high temperature oxidation resistance, consisting essentially of, by weight percent, about 14 to about 16% chromium, about 14 to about 17% nickel, 0.5 to about 3.0% manganese, about 4.0 to about 5.5% silicon, about 0.03 to about 0.10% carbon, about 0.03% maximum nitrogen, about 0.05% maximum phosphorus, about 0.05% maximum sulfur, and balance iron except for incidental impurities.

10 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195 10200 10205 10210 10215 10220 10225 10230 10235 10240 10245 10250 10255 10260 10265 10270 10275 10280 10285 10290 10295 10300 10305 10310 10315 10320 10325 10330 10335 10340 10345 10350 10355 10360 10365 10370 10375 10380 10385 10390 10395 10400 10405 10410 10415 10420 10425 10430 10435 10440 10445 10450 10455 10460 10465 10470 10475 10480 10485 10490 10495 10500 10505 10510 10515 10520 10525 10530 10535 10540 10545 10550 10555 10560 10565 10570 10575 10580 10585 10590 10595 10600 10605 10610 10615 10620 10625